

# UNITED STATES PATENT OFFICE.

JAMES MOSSMAN, OF CINCINNATI, OHIO, ASSIGNOR TO THE M. J. CUNNING COMPANY,  
OF CINCINNATI, OHIO, A CORPORATION OF OHIO.

## MARKING INK OR FLUID FOR USE ON EMBROIDERY FABRICS OR SHEETS.

1,159,857.

Specification of Letters Patent.

Patented Nov. 9, 1915.

No Drawing.

Application filed March 25, 1915. Serial No. 17,041.

To all whom it may concern:

Be it known that I, JAMES MOSSMAN, a citizen of the United States of America, and a resident of Cincinnati, in the county of Hamilton and State of Ohio have invented a certain new and useful Marking Ink or Fluid for Use on Embroidery Fabrics or Sheets, of which the following is a specification.

10 My composition relates to inks or colored fluids used in marking textile fabrics or the like in embroidery work and it consists of the following ingredients, combined in the proportions stated, viz:—coloring material one (1) ounce; linseed-oil, one and a half (1½) ounces; bees-wax, two (2) ounces; turpentine, one-fourth (¼) ounce. These ingredients must first be thoroughly dissolved together and then run through a grinding-mill, one or more times as required, for acquiring a smooth, freely-running, fluid mixture, free from lumps, grits, or heavy, coarse substance.

20 In using the above-named composition or marking-fluid a quantity of it is poured on a slab and a flat, straight-edged implement like a spud or scraper employed to carry and spread a suitable charge or supply to the surface of a perforated pattern sheet or 30 stencil containing the designs to be afterward made on the transfer or impression sheet that is laid on a table below, preferably in multiple or in a stack for speedy and convenient action in handling. Each 35 transfer-sheet thus produced is placed on the goods or fabric to be worked with the embroidery designs, and then the desired design is transferred or impressed on said fabric from the impression-sheet by means 40 of friction or heat, as conditions prescribe or permit.

The frictional method is preferred and

conducted by means of any suitable implement, or the thumb-nail of the operator if need be and found best adapted to the work 45 when it is desired to get the ink well set into the surface of the fabric. Heat may be used, however, when the transfer-sheet has been used a number of times and the impression becomes faint, and then the heat enables the further use of said transfer-sheet 50 a few more times with good effect.

I employ bees-wax in my composition as a color-carrier transfer body or medium and prefer it to any other medium for the reason that it assures a finer and more distinct, clean-cut line for the embroiderer to follow in working out the design on the goods or fabric no matter of what texture. The coloring-element preferred for use in 60 the composition herein is of a shade of blue that is commonly known as iridescent-blue, or one that has rainbow or prismatic effects, with the blue predominant.

I claim:

1. The herein-described composition of matter for use as a marking ink or fluid in the transfer or reproduction of designs on embroidery fabrics or sheets, consisting of a coloring-element, linseed-oil, bees-wax and 70 turpentine, substantially in the proportions described.

2. The herein-described composition of matter for use as a marking ink or fluid in the transfer or reproduction of designs on 75 embroidery fabrics or sheets, consisting of a coloring-element one ounce, linseed-oil one and one-half ounces, bees-wax two ounces, and turpentine one-fourth ounce, substantially as described.

JAMES MOSSMAN.

Witnesses:

JOHN ELIAS JONES,  
WILLIAM SCHUCHARDT.